

reduces the amount of carbon deposited on vital engine parts. The present invention is directed to a method of reducing the amount of carbon deposited on vital engine parts by adding a hydroperoxide to a fuel high in aromatic hydrocarbons.

It has now been found that the amount of carbon deposited on vital engine parts can be greatly reduced by adding 0.1 to 5% by weight of a hydroperoxide to a turbo-jet fuel high in aromatic hydrocarbons.

## UNITED STATES PATENT OFFICE

Patent No. 2,609,279, issued Sept. 2, 1952, to Kenneth G. Morris, Cranford, and Raymond A. Van Sweringen, Jr., Roselle Park, N. J., assignors to Standard Oil Development Company, a corporation of Delaware.

No Drawing. Application November 26, 1949,  
Serial No. 129,896

2 Claims. (Cl. 44—57)

1

This invention relates to fuels for turbo-jet engines and more particularly relates to a method for reducing the carbon deposition of turbo-jet fuel high in aromatic hydrocarbons.

Development of the aviation turbo-jet engine since its initial successful trials during the latter part of World War II has been very rapid. The advances have been spurred on by the potential high speed performance possibilities of jet propelled craft compared with the propeller driven type which attain their best efficiencies at lower air speeds.

Early aviation turbo-jet engines and most of those presently in use were designed to operate with a low aromatic, kerosene-type fuel almost identical with domestic kerosene. Combustor designs, which were developed originally by a cut-and-try method, have been adjusted to this fuel by subsequent designs until performance and maintenance for sea level and limited altitude operation are approaching satisfactory limits.

With the increased use of jet engines has arisen the logical question of fuel supply for probable expanding commercial requirements and for possible more immediate military emergencies. These supply requirements have necessitated institution of the present broad specifications for a 5-7 lb. RVP, 600° FEP fuel containing higher percentages of aromatics, olefins, and sulfur. Such liberalizing in petroleum fuel specifications will result in better than a three-fold increase in supplies with less problems in feed stock selection and segregation for the fuel supplier.

The changing of fuel specifications has imposed problems of engine deposition in present engine combustors.

It has now been found that the amount of carbon deposited on vital engine parts can be greatly reduced by adding 0.1 to 5% by weight of a hydroperoxide to a turbo-jet fuel high in aromatic hydrocarbons.

The following examples illustrate the advantages to be secured by the practice of the present invention:

TURBOJET FUEL

Kenneth G. Morris, Cranford, and Raymond A. Van Sweringen, Jr., Roselle Park, N. J., assignors to Standard Oil Development Company, a corporation of Delaware

RECEIVED  
SEARCHED  
INDEXED  
MAILED  
JULY 1952  
U. S. PATENT OFFICE  
REG. U. S. PAT. OFF.

2  
Example 1

A high aromatic jet fuel having the following inspection

|    |                                                                                                                                                                              |        |
|----|------------------------------------------------------------------------------------------------------------------------------------------------------------------------------|--------|
| 5  | Gravity                                                                                                                                                                      | 26.1   |
|    | Reid vapor pressure, p. s. i.                                                                                                                                                | —      |
|    | Flash point (Tag cc), °F.                                                                                                                                                    | 150    |
|    | ASTM distillation, °F.:                                                                                                                                                      |        |
| 10 | I. B. P.                                                                                                                                                                     | 347    |
|    | 10% —                                                                                                                                                                        | 378    |
|    | 50% —                                                                                                                                                                        | 383    |
|    | 90% —                                                                                                                                                                        | 393    |
|    | F. B. P.                                                                                                                                                                     | 425    |
|    | Freezing point, °F.                                                                                                                                                          | —10    |
| 15 | Corrosion test                                                                                                                                                               |        |
|    | Sulfur, weight percent                                                                                                                                                       | 0.026  |
|    | Aromatics, volume percent by ASTM                                                                                                                                            | 99     |
|    | ES-45                                                                                                                                                                        | —      |
|    | Bromine number, eg./g.                                                                                                                                                       | 0.3    |
| 20 | Viscosity, centistokes:                                                                                                                                                      |        |
|    | At —40° F.                                                                                                                                                                   | —      |
|    | At +100° F.                                                                                                                                                                  | —      |
|    | ASTM gum, mg./100 ml.                                                                                                                                                        | 18.9   |
|    | ACC. Army Gum Test, mg./100 ml.:                                                                                                                                             |        |
| 25 | 7 hours                                                                                                                                                                      | —      |
|    | 16 hours                                                                                                                                                                     | —      |
|    | Net heating value, B. t. u./lb.                                                                                                                                              | 17,775 |
| 30 | was burned in the General Electric I-40 single combustor engine with and without the addition of 2 weight percent cumene hydroperoxide and the following data were obtained: |        |

|                                     | Jet Fuel | Jet Fuel<br>+2%<br>Cumene<br>Hydro-<br>peroxide |
|-------------------------------------|----------|-------------------------------------------------|
| 35                                  |          |                                                 |
| Operating Conditions:               |          |                                                 |
| Air Rate, lb./sec.                  | 2.0      | 2.0                                             |
| Fuel Rate, lb./sec.                 | 0.04     | 0.04                                            |
| Comb. Inlet Air Press., in. Hg abs. | 48       | 48                                              |
| Comb. Inlet Air Temp., °F.          | 300      | 300                                             |
| Time, hrs.                          | 4.25     | 4.25                                            |
| Carbon Deposition, g.:              |          |                                                 |
| Liner                               | 48       | 16.1                                            |
| Dome                                | 3.0      | 3.2                                             |
| Spark Plug                          | 1.6      | 0.6                                             |
| Total                               | 52.6     | 19.9                                            |

The above data show that the quantity of carbon was reduced 62%. A check run showed about the same percentage of carbon reduction.

*Example II*

A test similar to that of Example I was carried out using a non-aromatic fuel having the following inspection:

|                                   |        |    |
|-----------------------------------|--------|----|
| Gravity, °API                     | 48.0   | 10 |
| Reid vapor pressure, p. s. i.     | 4.9    |    |
| Flash point (Tag cc.), °F.        |        |    |
| ASTM Distillation, °F.:           |        |    |
| I. B. P.                          | 116    |    |
| 10%                               | 154    |    |
| 50%                               | 391    | 15 |
| 90%                               | 510    |    |
| F. B. P.                          | 576    |    |
| Freezing point, °F.               | < -76  |    |
| Corrosion test                    | Passes | 20 |
| Sulfur, weight percent            | 0.308  |    |
| Aromatics, volume percent by ASTM |        |    |
| ES-45                             | 28.3   |    |
| Bromine number, cg./g.            | 5.87   |    |
| Viscosity, centistokes:           |        |    |
| At -40° F.                        | 3.928  |    |
| At +100° F.                       | 0.9715 |    |
| ASTM Gum, mg./100 ml.:            |        |    |
| 7 hrs.                            | 18.0   |    |
| 16 hrs.                           | 21.5   | 30 |
| Net heating value, B. t. u./lb.   | 18,651 |    |

When this fuel was burned with and without the addition of 2 weight percent of cumene hydroperoxide, it was found that the cumene hydroperoxide had substantially no effect on the carbon formation as shown in the following table:

The above examples show that the addition of cumene hydroperoxide is effective in reducing the carbon deposition tendency of a jet fuel only when it contains a very large amount of aromatics.

5

The nature of the present invention having thus been described, what is claimed as new and useful and desired to be secured by Letters Patent is:

1. A fuel for use in turbo-Jets in which the oxygen required for combustion of the fuel is supplied by air, said fuel consisting essentially of a liquid hydrocarbon composition containing at least 50% by volume of aromatic hydrocarbons and 0.1 to 5% by volume of cumene hydroperoxide.

2. Composition as defined by claim 1 wherein the amount of cumene hydroperoxide present is about 2% by volume.

KENNETH G. MORRIS.

RAYMOND A. VAN SWERINGEN, JR.

REFERENCES CITED

The following references are of record in the file of this patent:

UNITED STATES PATENTS

| Number    | Name           | Date          |
|-----------|----------------|---------------|
| 1,766,501 | Buerk          | June 24, 1930 |
| 2,403,772 | Vaughan et al. | July 9, 1946  |
| 2,472,152 | Farkas         | June 7, 1949  |
| 2,534,309 | Sheffield      | Dec. 19, 1950 |

FOREIGN PATENTS

| Number  | Country       | Date         |
|---------|---------------|--------------|
| 476,227 | Great Britain | June 4, 1937 |

| Run No. | Fuel Used                      | Air Rate<br>lb./sec. | Air/Fuel<br>Ratio | Length<br>of Run<br>Hrs. | Com-<br>bustor<br>Inlet<br>Air<br>Temp.,<br>°F. | Com-<br>bustor<br>Inlet<br>Air<br>Press.,<br>p.s.i. | Fuel<br>Con-<br>sumed,<br>g. | Carbon Deposit, g. |       |       |
|---------|--------------------------------|----------------------|-------------------|--------------------------|-------------------------------------------------|-----------------------------------------------------|------------------------------|--------------------|-------|-------|
|         |                                |                      |                   |                          |                                                 |                                                     |                              | Dome               | Liner | Total |
| 1.      | Non-aromatic                   | 2.0                  | 50                | 4.25                     | 300                                             | 48                                                  | 278                          | 2.9                | 8.5   | 11.4  |
| 2.      | do                             | 2.0                  | 50                | 4.25                     | 300                                             | 48                                                  | 278                          | 2.5                | 7.5   | 10.0  |
| 3.      | do                             | 2.0                  | 50                | 4.25                     | 300                                             | 48                                                  | 278                          | 1.5                | 7.0   | 8.5   |
| 4.      | +2% Cumene Hydro-<br>peroxide. | 2.0                  | 50                | 4.25                     | 300                                             | 48                                                  | 278                          | 3.4                | 11.0  | 14.4  |